

## UNITED STATES PATENT OFFICE

2,274,676

## LUBRICANT CONTAINING LITHIUM SALTS

Clarence E. Earle, Washington, D. C.

No Drawing. Application November 4, 1940,  
Serial No. 364,249

10 Claims. (Cl. 252—56)

(Granted under the act of March 3, 1883, as  
amended April 30, 1928; 370 O. G. 757)

This invention relates to new and improved lubricating compositions containing lithium salts of various organic acids.

It is the object of this invention to provide lubricating compositions having a suitable oil base and a consistency that may be varied to suit different uses by the addition of lithium salts.

My copending application, Ser. No. 328,095, filed April 5, 1940, discloses the highly beneficial results arising from incorporating lithium soaps of the higher fatty acids in lubricating oils, both in mineral and in non-drying vegetable oils.

I have found that the use of lithium soap or salts of soap forming higher fatty acids in the production of lubricating greases gives the greases entirely different properties from those obtained by the use of the other alkali metal salts. The greases produced by my method are water resistant, whereas the other alkali salts do not give such a property. My lithium soap greases withstand temperatures greatly in excess of those containing other alkali metal salts. The properties of these improved lubricating greases are not only widely different from the other alkali metal soap types but also they are much more stable to temperature and pressure, both chemically and physically.

Suitable oils may be created with lithium salts to produce lubricants having consistencies ranging from viscous oil to grease-like structures. Among the lithium compounds so used are the lithium salts of acetic, butyric, ethyl butyric, ethyl hexoic and caproic acid. These lithium salts can be, when added to or produced by reactions in mineral or non-drying vegetable oils, in quantities from 4% to 40% by weight, give smooth homogeneous compositions that have high heat resistance, excellent water resistance and good cold operating properties.

In its broad aspects the subject matter of this present application is similar to that of my copending application, Serial No. 364,248, filed of even date herewith. Specifically, this present application is limited to the lithium salts of acetic and caproic acids.

The invention herein described and claimed

may be manufactured and used by or for the Government of the United States of America for governmental purposes without the payment of any royalties thereon or therefor.

I claim:

1. Lubricating compositions, comprising a lithium salt of an acid from the group consisting of acetic and butyric acids and an oil from the group consisting of mineral and non-drying vegetable oils, said salt being present in quantities of from 4% to 40%.

2. Lubricating compositions, comprising a lithium salt of an acid from the group consisting of acetic and butyric acids and an oil from the group consisting of mineral and non-drying vegetable oils, said salt being present in quantities sufficient substantially to thicken said oil.

3. Lubricating compositions, comprising mineral oil and a lithium salt of acetic acid in quantities of from 4% to 40%.

4. Lubricating compositions, comprising mineral oil and a lithium salt of acetic acid in quantities sufficient substantially to thicken said oil.

5. Lubricating compositions, comprising a non-drying vegetable oil and a lithium salt of acetic acid in quantities of from 4% to 40%.

6. Lubricating compositions, comprising a non-drying vegetable oil and a lithium salt of acetic acid in quantities sufficient substantially to thicken said oil.

7. Lubricating compositions, comprising mineral oil and a lithium salt of butyric acid in quantities of from 4% to 40%.

8. Lubricating compositions, comprising mineral oil and a lithium salt of butyric acid in quantities sufficient substantially to thicken said oil.

9. Lubricating compositions, comprising a non-drying vegetable oil and a lithium salt of butyric acid in quantities of from 4% to 40%.

10. Lubricating compositions, comprising a non-drying vegetable oil and a lithium salt of butyric acid in quantities sufficient substantially to thicken said oil.

CLARENCE E. EARLE.